

J. A. NOBLE.  
PREPARATION OF ADHESIVE SURFACES.  
APPLICATION FILED JULY 19, 1920.

1,361,894.

Patented Dec. 14, 1920.

Fig. 1



Fig. 2



Fig. 3



INVENTOR.  
James A. Noble  
BY  
G. D. Church  
his ATTORNEY

# UNITED STATES PATENT OFFICE.

JAMES A. NOBLE, OF ROCHESTER, NEW YORK.

## PREPARATION OF ADHESIVE SURFACES.

1,361,894.

Specification of Letters Patent.

Patented Dec. 14, 1920.

Application filed July 19, 1920. Serial No. 397,328.

To all whom it may concern:

Be it known that I, JAMES A. NOBLE, of Rochester, in the county of Monroe and State of New York, have invented certain new and useful Improvements in the Preparation of Adhesive Surfaces; and I do hereby declare the following to be a full, clear, and exact description of the same, reference being had to the accompanying drawings, forming a part of this specification, and to the reference numerals marked thereon.

My improvements are particularly applicable to prepared fabrics that are often made as a substitute for or imitation of leather and consist of a woven body portion having a dried coating on one side to provide the smooth, flexible and waterproof or other finished surface and the tacky surface on the other side consisting of a coating of a more or less permanently sticky adhesive, through the medium of which the fabric is applied to objects that it is desired to trim, or cover over. Cheap material of this kind is ordinarily difficult to handle because of the tacky substance adhering so readily when doubled upon itself or placed in contact with adjacent sheets, and it is the object of my invention to render this tacky surface temporarily non-adhesive so that the sheets may be handled with greater rapidity and facility. It is the further object of my invention, however, not to thereby impair the ultimate value of the tacky surface as an adhesive. To these and other ends the invention resides in certain improvements and combinations of parts, all as will be hereinafter more fully described, the novel features being pointed out in the claims at the end of the specification.

In the drawings:

Figure 1 is a plan view of a sheet of material constructed in accordance with and illustrating one embodiment of my invention.

Fig. 2 is an enlarged sectional view thereof, and

Fig. 3 is a similar sectional view showing the addition to the surface of a coating of cement in the final use thereof.

Similar reference numerals throughout the several views indicate the same parts.

Material of the nature I have mentioned consisting of a fabric body, an outer finished 55 coating and an inner tacky coating is largely

used as a finishing material in the manufacture of camera bellows, and I have shown in the drawing a blank cut for this purpose. The respective coatings are usually of a rubber, cold tar, or similar derivation, and after the fabric body of the bellows has been formed and stiffened with paper at the proper points, the finishing covering is applied to the rough surface of fabric and paper by adding a coating of ordinary rubber cement to the tacky surface and pressing it thereon. I have discovered that by initially powdering the tacky surface with certain materials in a finely comminuted and dry or solid state, such surface is rendered temporarily non-adhesive and the sheets may be piled one upon the other and carelessly handled without adhering to each other or to other objects, and yet when the cement is applied the film of powder is eradicated as such and in no way interferes with the adhesiveness which is immediately restored, if not increased.

The substances I have used with success, as the powdering medium, are themselves adhesives, and consist of gelatinous or animal glue, vegetable glue, including broken down starch or dextrin compounds, and a commercial glue known as "Motan" glue, the composition of which is not known to me but which I understand to be a by-product from the waste sulfite liquors produced in paper manufacture. It is a resinous product and readily admits of pulverization. These substances, in powdered form, are simply dusted upon the surface until its adhesiveness has disappeared.

When it is desired to convert the surface back to its tacky consistency a film of rubber cement is spread thereon in the customary way, and I find that it has the property of either taking the glue into solution, or at least forming therewith a colloidal solution, such action being equivalent so far as the desired results are concerned to an ordinary solution. The glue mixes in the fluid cement in particles of colloidal size, thus eliminating the resistant effect to adhesion. The rubber cement may be the usual composition of Para rubber dissolved in carbon bisulfid and benzin or naphtha (including gasolene) as a volatile solvent.

Of the substances enumerated I have obtained the best results with Motan glue and a cement of the nature just mentioned.

My invention is of great utility not only in packing, storing and shipping adhesive sheets and the like, but in handling the same in processes of manufacture. For instance, 5 in the manufacture of camera bellows as outlined, the tacky covering must be trimmed in various ways at different stages in the formation of the bellows, and the temporarily inert or powdered and non-adhesive surface 10 is much more readily acted upon in this way than one that is sticky and quick to adhere to any surface with which it is brought in contact.

In the accompanying drawing 1 indicates 15 generally a blank of flexible imitation leather cloth cut to a form for application to a camera bellows. The body of the cloth in the sectional views is indicated at 2, the outer finished coating at 3, and the tacky or 20 adhesive coating at 4. Powdered on the latter are the particles of glue shown at 6 in Fig. 2. In Fig. 3 these particles are shown to have disappeared in the film of rubber cement 5 that has been applied to the tacky 25 coating 4.

I claim as my invention:

1. The method of rendering a tacky surface temporarily non-adhesive which consists in powdering such surface with an adhesive in solid form.

2. The method of rendering a tacky surface temporarily non-adhesive which consists in powdering such surface with another adhesive in solid form and insoluble in the 35 tacky substance.

3. The method of rendering a tacky surface temporarily non-adhesive which consists in powdering such surface with an adhesive in solid form, and then applying to 40 the surface, preparatory to its use, a cement

which is a solvent for the powdered adhesive.

4. The method of rendering a tacky surface temporarily non-adhesive which consists in powdering such surface with a glue 45 insoluble in the tacky substance.

5. The method of rendering a tacky surface temporarily non-adhesive which consists in powdering such surface with Motan 50 glue.

6. The method of rendering a tacky surface temporarily non-adhesive which consists in powdering such surface with Motan glue, and then applying to the said surface, 55 preparatory to its use, a rubber cement.

7. The method of rendering a tacky surface temporarily non-adhesive which consists in powdering such surface with another adhesive in solid form and insoluble in the tacky substance, and then applying to the 60 surface, preparatory to its use, a cement which is a solvent for the powdered adhesive and which combines adhesively with the tacky substance.

8. As an article of manufacture, a flexible 65 sheet adapted to be joined to another object by adhesion and provided with a tacky coating, the surface of the latter being covered with a powdered adhesive.

9. As an article of manufacture, a flexible 70 sheet adapted to be joined to another object by adhesion and provided with a tacky coating, the surface of the latter being powdered with a glue insoluble in the tacky substance.

10. As an article of manufacture, a flexible 75 sheet adapted to be joined to another object by adhesion and provided with a tacky coating, the surface of the latter being powdered with Motan glue.

JAMES A. NOBLE.